

Jan. 7, 1930.

A. L. SMITH

1,742,618

OVERLAY SHEET AND METHOD OF PRODUCING THE SAME

Filed Jan. 17, 1929



Fig. 1.



Fig. 2.



Fig. 3.

Inventor.  
Arthur L. Smith  
By S.H. Hammann  
Atty.

Patented Jan. 7, 1930

1,742,618

# UNITED STATES PATENT OFFICE

ARTHUR L. SMITH, OF BOSTON, MASSACHUSETTS, ASSIGNOR TO CAMEO OVERLAY CORPORATION, OF CAMBRIDGE, MASSACHUSETTS, A CORPORATION OF MASSACHUSETTS

## OVERLAY SHEET AND METHOD OF PRODUCING THE SAME

Application filed January 17, 1929. Serial No. 333,115.

This invention relates to overlay sheets which are usually employed on the cylinders or platens of printing presses beneath a tympan, for the purpose, primarily, of improving the results secured by the printing operation from half-tone cuts, the preparation and adjustment of such sheets being an operation known as "make ready".

More particularly the invention relates to that type of overlay sheets in which a powdered material is placed on a freshly printed proof sheet, so that a portion of the material will be retained by the wet ink when the surplus material is shaken off the sheet, a further operation usually being necessary to attach the material to the sheet which was retained by the ink, so that certain portions of the sheet become permanently embossed.

The above type of sheet is to be distinguished from those types in which portions of the sheet are actually cut out, or built up by pasting on pieces of paper, or those in which the proof is printed on specially prepared paper, which later is etched in a suitable bath. Overlay sheets made by the "cut out" method are expensive and often require a high degree of skill in their preparation, but both methods are disadvantageous in certain respects, for various reasons, one of

the principal of which is the length of time required to make the sheets, for the time required to make an overlay sheet is often a much more important consideration than the labor cost of making it, as the press on which the overlay sheet is to be used must be idle while the sheet is being prepared, and there is often a demand that the printing operation be performed as quickly as possible.

One of the principal defects in the embossed overlay sheets, made by processes which have been previously employed, is due to the fact that the extent of the embossment of any portion usually fails to be even approximately in proportion to the depth of the shadows in the picture to be reproduced, so that, when the picture is printed, the desired gradation of the different tones are not secured. Another defect is due to the use of various adhesive and liquid coatings to secure embossing material to the sheet, which are likely to cause expansion or contraction of the sheet as a whole, so that it becomes practically impossible to position the overlay sheet in correct relation to the printing characters. Adhesives are also usually ineffective in securing the embossment to the sheet, so that the embossment has been coated with shellac, silicate of soda and other self hardening adhesives to secure it, and where the overlay is coated with such materials, a hard, brittle, and somewhat glassy surface is usually produced thereon which is objectionable for several reasons, some of which are that the pressure of the cylinder on the bed tends to crush the embossment, so as to destroy it, or reduce its effectiveness to such an extent that the sheet becomes practically useless after it has been used for a short portion of the desired run, also, such a sheet is liable to slip slightly out of position on the cylinder, and, if a sheet slips even slightly, the printed results are not only likely to be unsatisfactory, but serious damage is likely to be caused to a plate or cut.

Also, in producing an embossed overlay sheet by many of the previously employed processes, it has been necessary to use a special ink, usually of highly adhesive nature, in making the proof, and this necessity has been found to be highly objectionable, in practice, as it involves changing the ink in the press, to strike off the single proof, and then changing back to regular ink and cleaning the plate or type.

The objects of my invention are to produce an overlay sheet of the embossed type and a process of making the same including a composition of substances to be employed in the production thereof, which will obviate many of the objections to overlay sheets of this type, particularly by producing sheets which will be as heavily embossed on the low lights, or solid tones, as may be necessary to produce solid black, or other solid color on the corresponding parts of the matter to be reproduced, and which will be less heavily embossed on the middle and grey tones, so that the desired gradation of shade will be secured on these portions of the printed reproduction, and which will be entirely unembossed on the high light portions, so that they will not

be inked at all in printing and the pressure on these portions of a plate or cut will not be increased.

Also to provide a process which will make it unnecessary to use a special ink in striking off the proof, and will permit the use of any ink which happens to be supplied to the press.

Other objects are to provide a process of producing an embossed overlay sheet which will not necessitate the use of any material in liquid form, but will permit the sheet to be kept dry throughout the process, so that there will be no action tending to cause the sheet as a whole to expand or shrink. Also to provide a process which will merely necessitate heating the sheet to fix the embossment thereto and which, on fusion of the material, will nevertheless prevent liquid of fusion from flowing over the lines between the different shades, so as to cause distortion of these lines, and will also cause the edges of the more heavily embossed portions to be beveled, so that the increased pressure secured by such portions will not increase the pressure on adjacent portions.

Also to produce an embossed overlay sheet which will normally have a somewhat roughened, pebbly, or corrugated surface, but which is also resilient, so that it may be pressed flat while under the direct pressure of the cylinder, but will resume its pebbly surface when the pressure is removed, and which will normally frictionally engage the tympan, by causing slight indentations therein, so that all possibility that the overlay sheet will slip out of position on the cylinder is obviated.

Also to produce a sheet which is perfectly flexible as well as resilient, so that the sheet will not be detrimentally affected by the action of the cylinder in pressing it against the bed, permitting the number of reproductions which may be printed to be practically unlimited.

Also to provide a composition of substances to be employed in the production of an embossed overlay sheet which will enable a sheet having the advantageous characteristics above referred to, to be produced without the employment of the highly skilled labor usually necessary in make-ready, and which will enable uniformity of results to be secured.

I accomplish these objects by providing a powder for embossing the overlay sheet which is composed of a mixture of substances consisting principally, or wholly, of certain forms of gum which have been reduced, by a screening operation, to two or more sizes, the larger of which, when applied to the proof, will adhere to the more heavily inked portions, or solid tones of the proof, without adhering to the less heavily inked portions to a substantial extent, and the smaller of which will adhere to all portions which have been

inked and has not been absorbed by the paper or the coating thereon.

Also by providing an embossing powder which is composed of gums having different fusing points, the gum from which the larger sized grains are formed being of a resilient nature and having the highest fusing point, and the material from which the smaller grains are formed having a relatively low fusing point, so that the smaller grains may become fused first, when the sheet is heated, and will penetrate the paper and then, on further heating, its larger grains will become slightly fused on their surfaces and united to the mass already fused, so that all the material, including the larger grains, will be fixed on the sheet and practically integrally attached thereto without fusing said larger grains sufficiently to impair their resiliency.

Also by including in the embossing powder small grains of an astringent material, which is thoroughly mixed therewith and has a low fusing point, so that it will become fused at approximately the time when the other smaller grains become fused and which will act to prevent the fused material from spreading over the sheet and flowing beyond the lines of the shaded portion of the sheet to which the material was applied and will also act to draw in the unfused, or partly fused grains from said lines, so that the margins of the embossed portions will be slightly beveled.

The more specific details as to the manner in which the above described, as well as other advantageous results, are secured, are more fully described in the following specification, in connection with the accompanying drawings, in which:

Figs. 1 and 2 are greatly enlarged sectional views of an overlay sheet illustrating different steps in my herein described process.

Fig. 3 is a sectional view on an enlarged scale, showing the application to a press cylinder.

While the overlay sheet may be employed in connection with printing presses of different types, for the purpose of convenience in description, the type of press which will be referred to hereinafter comprises a reciprocating bed, on which the printing characters are mounted, and a cylinder, having a tympan thereon, composed of several paper sheets.

In producing an embossed overlay sheet embodying my invention, I preferably employ a sheet of good quality chalk coated paper, which in many instances, is preferably coated with pummy talc, so that it will absorb any small amount of ink which may be applied by the high light portions of the printing characters, and prevent subsequent adhesion of the embossing powder to such portions, thereby avoiding the necessity of removing the embossing material from such portions, as these portions should not be

inked at all in printing and the pressure of the cylinder thereon should not be in any way increased by the presence of the overlay. A proof of the printing characters is then taken off on the sheet with the ordinary ink with which the press is supplied, and an impression is also taken on the tympan for positioning purposes. The proof sheet will be most heavily inked on the solid tone portions of the proof and more lightly inked on the middle and grey tone portions thereof, the remainder of the process, briefly outlined, being as follows:

The embossing powder, hereinafter more specifically described, is then dusted or "run" over the freshly printed surface, so that it comes in contact with all parts thereof, and then the surplus powder is shaken off, by suspending it from one edge and tapping it sharply, so that the only grains of the powder which remain are those which have come directly in contact with the wet ink. The sheet is then held horizontally with its coated side up, and heated on its under side, preferably by holding it over an electric heater, until all the grains which have adhered to the sheet take on a glazed appearance, and then the sheet is ready to be placed on the press cylinder beneath the tympan, in register with the impressions which has been made thereon.

As the result of much experimentation, I have ascertained, that, in employing an embossing powder for this purpose, particularly when largely composed of substances of the gumming nature which I employ, grains of a certain size will adhere to the more heavily inked surfaces, but will not be retained to any substantial extent by the more lightly inked portions, when the surplus powder is shaken off as above described, and that grains of a smaller size will adhere under these conditions to both the heavily and lightly inked surfaces. That is, I have ascertained that a definite relation, within certain limits, exists between the size of the grains and the extent to which a surface must be inked to retain the grains. I have further ascertained that grains of a size which will adhere to the middle and grey tone surfaces will not sufficiently emboss the solid tone portions, as practically no grains will adhere to the sheet which do not come into actual contact with the ink.

To secure, as nearly as practicable, the desired gradations of embossment, and consequently the desired gradations of tone in the printed picture, I provide a compound composed of a mixture of grains of suitably graded sizes in predetermined proportion, the larger of which will ordinarily adhere to the more heavily inked surfaces only. Under many conditions it is unnecessary to employ grains of more than two sizes in the compound, although, under some conditions

the employment of grains of an intermediate size is desirable and under other conditions I have found it desirable to employ grains of as many as six different sizes. For ordinary purposes I provide a compound which preferably comprises a suitable proportion of a gum known commercially as "copal gum," which fuses at approximately 200° C., and which has been passed through an 80 mesh screen, and a suitable proportion of a commercial gum, known as dammar gum, which fuses at about 120° C. and which has been passed through a 150 mesh screen. While I consider these sizes particularly desirable, advantageous results may be secured with grains of these materials which approximate thereto, as the grains of each size may be made slightly larger or smaller without materially affecting the results, although the approximate relative proportion of the sizes should be maintained. When applied to the freshly printed sheets the larger grains of copal gum will ordinarily adhere to the solid tone portion only of the picture, and the smaller grains will fill in the spaces therebetween, as indicated on a greatly enlarged scale in Fig. 1, in which a sheet *a* is indicated as having both the larger sized grains *b* and smaller sized grains *c* adhering to the heavily inked surface portion *d* of the sheet and the smaller sized grains *e* adhering to the less heavily inked surface *e*.

I further include in the compound a suitable quantity of either Bergundy pitch, or carnauba wax, the last named being preferable, as it is the least expensive. This substance is reduced to approximately the same degree of fineness as the dammar gum, and is thoroughly mixed therewith. The melting points of the carnauba wax is approximately 85° C., so that, when the sheet is heated, both the dammar gum and the carnauba wax will become completely fused before the copal gum is fused to any substantial extent, particularly also because they have been reduced to a greater degree of fineness.

As a result of the heating operation, the carnauba wax will fuse first and will penetrate the paper and the dammar gum will fuse immediately thereafter, or at practically the same time, so that the grains of copal gum will be surrounded and more or less coated by this fused material. On still further heating, the surfaces of the grains of copal gum will be slightly fused and will thus unite with the material already fused and thus will be securely attached to the paper on cooling. To secure this result, the heating operation is continued until the powder on the sheet assumes a glossy appearance, which is due to the presence of the dammar gum, and provides an accurate guide to the operator, so that, with reasonable care, over heating, or heating to an extent sufficient to destroy the resiliency of the copal gum will be prevented,

while sufficient heat will be supplied to fix the materials to the sheet, as indicated in Fig. 2.

However, if these ingredients alone were employed in the manner above described, the fused material would flow over the lines between the portions having different degrees of shading or tone, with the result that these lines would be distorted, so that the results would be unsatisfactory.

I have discovered that this difficulty may be entirely avoided by also combining with the other substances above specified, a suitable quantity of a substance which will act as an astringent and has a low melting point, for example:—gum sumac, tannic acid, or alum. Of these substances the gum sumac is considered preferable. This substance is also reduced to approximately the same degree of fineness as the dammar gum and is thoroughly mixed with all the substances above specified. It also has a fusing point which approximates to that of dammar gum and the carnauba wax and, as it is reduced to the same fineness as these substances, will begin to fuse at practically the same time that the other smaller size grains begin to fuse. As soon as the astringent, or gum sumac begins to fuse, it also begins to contract and thus contracts the liquid formed by the fusion of the other substances with which it is mixed, and acts to draw together the unfused or slightly fused grains of copal gum, so that the spreading out of the fused mass or the grains beyond the space on which they are deposited, is prevented. The material which is deposited on any portion of the sheet, which is fused, is contracted and the unfused or partly fused grains are drawn together, so that the material, as a whole, is slightly drawn away from the edge of the space on which it was deposited, and, as a result, the embossment on the finished overlay sheet is slightly beveled or rounded at the line between the solid tone of the picture and the adjacent tones of lighter shade, as indicated in Fig. 2. This result is important, not only for the reason that the embossing substance is prevented from spreading onto adjacent shadows of less depth, but also because, when in use, the increased pressure on any portion due to the embossment might cause an increase of pressure on adjacent portions, if the embossment retained its full thickness to the edge, and, as a result, the line between the corresponding adjacent portions of the printed picture would be distorted, but if the edges of the embossments are slightly beveled, as above described, the possibility of such an occurrence is avoided.

The ingredients of the compound in the approximate portions which I preferably employ in securing the above described results are as follows:

45% copal gum, screened to 80 mesh, and fusing at about 200° C.

35% dammar gum, screened to 150 mesh, and fusing at about 120° C.

8% gum sumac, screened to 150 mesh, and fusing at about 120° C.

12% carnauba wax, screened to 150 mesh, and fusing at about 85° C.

It will be understood that various other forms of gums, resins and astringents, may be substituted for those above specified, as any of these substances having similar characteristics are considered to be equivalents.

The primary functions of the different ingredients above specified are as follows:

The copal gum provides a heavy embossment for the solid tones and a resilient pebbly surface.

The carnauba wax, by melting first, penetrates the paper and serves as an anchor for the embossment.

The dammar gum, by melting immediately thereafter, acts as a binder, attaching itself to the penetrating wax and to the fused surface of the copal gum grains and also serves as an embossment for the middle tones.

The gum sumac acts as an astringent to prevent the fused material from flowing over the lines between different shade tones and to draw in the grains so that the edges of each embossment will be slightly beveled.

An overlay sheet made by the above described process is advantageous for various reasons:

As the grains of the copal gum retain their shape and resiliency to a large extent, the surface of the embossed portions have a rough, and somewhat pebbly appearance, so that when the sheet *a* is placed in position on the cylinder *f* beneath the tympan *g*, as shown in Fig. 3, this roughened surface will become, by reason of the pressure on the tympan, slightly indented in the latter, or will have a strong frictional engagement therewith, so that all possibility of slipping of the overlay sheet on the cylinder will be prevented. Under the action of the cylinder in pressing the paper to be printed against the printing characters, as *h*, the embossment on the overlay sheet will be pressed flat by the cylinder at the point of contact of the latter with the bed, but, as soon as the pressure on any portion of the embossment is removed, it will be restored to normal by its resiliency, as indicated in Fig. 3. The heavy compression to which the overlay sheet is subjected by the cylinder has no detrimental effect thereon, as the embossment on the sheet is both resilient and flexible, so that the sheet may be used practically indefinitely, or as long as it would be likely to need to be used for any run of the press.

The extent of the embossment on the different tones of the proof sheet may be somewhat varied by varying the sizes of the grains in the embossing powder, but where extra heavy pressure on the printing characters or

plate is desired, two overlay sheets may be employed, one being arranged over the other in register therewith.

The process of making the sheet may be performed in a relatively short time as compared with other processes of which I am aware, and as the sheet is not at any time subjected to treatment with any liquid, it remains fixed in all its surface dimensions.

10 The overlay sheet hereinbefore described while primarily desirable in connection with printing from half-tone cuts, or plates, and enabling results to be secured which, so far as I am aware, cannot be secured by any of 15 the other methods herein referred to, is also advantageous in printing from type where heavy and light characters are to be printed.

I claim:

1. The method of making an embossed 20 overlay sheet for makeready in printing which consists in covering the freshly inked surface of a proof sheet with an embossing powder composed of a mixture of grains of a suitable material composed of a predetermined proportion of grains of a size which 25 will be retained to a substantial extent by the more heavily inked portions only of the sheet, and a predetermined proportion of grains of smaller size which will be retained by both 30 the heavily and lightly inked portions, shaking off the surplus powder and then fixing the powder which has been retained to the sheet.

2. The method of making an embossed 35 overlay sheet for makeready in printing, which consists in covering the freshly inked surface of a proof sheet with an embossing powder composed of a mixture of grains of gum composed of a predetermined proportion 40 of grains of a size which will be retained to a substantial extent by the more heavily inked portions only of the sheet, and a predetermined proportion of grains of gum of a relatively small size which will be retained by 45 both the heavily and lightly inked portions thereof, then shaking off the surplus powder and then heating the sheet to fix the remaining powder thereto.

3. The method of making an embossed 50 overlay sheet for makeready in printing which consists in covering the freshly inked surface of a proof with a powdered gum composed of a mixture of grains, a predetermined proportion of which are graded to a 55 size which will be retained by the more heavily inked portions only of the sheet and a predetermined proportion of which are graded to a relatively small size, and will also be retained by more lightly inked portions, shaking off the surplus material, and heating the sheet to fuse the smaller grains and by their fusion to fix the larger grains to the sheet.

4. The method of making an embossed 60 overlay sheet for makeready in printing

which consists in covering the freshly inked surfaces of a proof with a powdered resilient gum composed of grains of a size sufficient to be retained by the more heavily inked portions of the sheet and by a powdered gum the grains of which fuse at a lower temperature than that at which said larger grains fuse, shaking off the surplus material, and heating the sheet to fuse the smaller grains and by their fusion to fix the larger grains to the sheet.

5. The method of making an embossed overlay sheet for makeready in printing which consists in covering the freshly inked surface of a proof sheet with an embossing powder comprising a resilient gum composed of grains of a size which will be principally retained by the more heavily inked portions only of the sheet and mixed with a gum composed of grains of relatively small size, shaking off the surplus powder, heating the sheet to fuse the smaller grains and cause the fused material to become attached to the sheet and become fused to the larger grains to fix the latter on the sheet.

6. The method of making an embossed overlay sheet for makeready in printing which consists in covering the freshly inked surface of a proof sheet with an embossing powder comprising a resilient gum composed of grains of a size which will be retained principally by the more heavily inked portions only of the sheet and a substance composed of relatively small grains and having a substantially lower melting point than that of the larger grains, shaking off the surplus powder, heating the sheet to fuse the smaller grains and cause the fused material to become attached to the sheet and to cause surface fusion of the larger grains to fuse the latter to the fused material and to the sheet.

7. The method of making an embossed overlay sheet for makeready in printing which consists in covering the freshly inked surface of a proof sheet with an embossing powder comprising a mixture of a resilient gum composed of grains of relatively large size and high fusing point which will adhere principally to the more heavily inked portions only of the sheet and a gum composed of grains of relatively small size and low melting point and heating the sheet to fuse the smaller grains and fix the larger grains to the sheet without substantial fusion thereof.

8. The method of making an embossed overlay sheet for makeready in printing which consists in covering the freshly inked surface of a proof sheet with an embossing powder comprising a mixture of a resilient gum composed of grains of relatively large size and high fusing point which will adhere principally to the more heavily inked portions only of the sheet and two similar materials composed of grains of relatively small

70

75

80

85

90

95

100

105

110

115

120

125

130

- size, one of which has a relatively low fusing point and the other a fusing point intermediate that of the other materials, shaking off the surplus material, heating the sheet to fuse the grains of lower fusing points successively to permit the material first fused to penetrate the sheet and to surround the larger grains with the fusion of both materials and fix the larger grains to the sheet.
5. 9. The method of making an embossed overlay sheet for makeready in printing which consists in covering the freshly inked surface of a proof sheet with a powder comprising a fusible granular embossing material mixed with a fusible granular astringent material and then heating the sheet to fix the powder thereto.
10. 10. The method of making an embossed overlay sheet for makeready in printing which consists in covering the freshly inked surface of a proof with a fusible embossing powder comprising a powdered gum mixed with a powdered astringent and heating the powder retained by the ink to fix it to the sheet.
15. 11. The method of making an embossed overlay sheet for makeready in printing which consists in covering the freshly inked surface of a proof with an embossing powder comprising a powdered gum having a relatively high fusing point and mixed with a powdered astringent having a lower fusing point, and heating the powder retained by the ink to fix it to the sheet.
20. 12. The method of making an embossed overlay sheet for makeready in printing which consists in covering the freshly inked surface of a proof sheet with an embossing powder comprising a powdered gum divided into grains of a relatively large size mixed with an astringent having a substantially lower melting point than that of the gum and divided into grains of relatively small size, and then heating the sheet to fuse the astringent and then fuse the gum to the sheet.
25. 13. The method of making an embossed overlay sheet for makeready in printing which consists in covering the freshly inked surface of a proof sheet with an embossing powder comprising a powdered gum divided into grains of a relatively large size mixed with a gum and an astringent, both of which have substantially lower melting points than that of the gum from which the larger grains are formed, and are divided into relatively small grains, and then heating the sheet to fuse the smaller grains and fuse the larger grains to the sheet.
30. 14. The method of making an embossed overlay sheet for makeready in printing which consists in covering the freshly inked surface of a proof sheet with an embossing powder containing a powdered gum and a powdered astringent, shaking off the surface plus powder and then heating the sheet to fuse the gum sufficiently to fix it to the sheet and by the action of the astringent when heated to draw the gum away from the margin of the inked spaces to which has adhered.
35. 15. An embossing powder for making overlay sheets for makeready in printing which comprises two powdered gums, one being composed of large grains and the other of relatively small grains.
40. 16. An embossing powder for making overlay sheets for makeready in printing which comprises two powdered gums, one being composed of large grains having a high melting point and the other of relatively small grains having a relatively low melting point.
45. 17. An embossing powder for use in making an embossed overlay sheet, which consists of powdered gum which has a tendency to flow on the sheet when fused, mixed with a powdered astringent which has the property of counteracting said tendency of the gum.
50. 18. An embossing powder for use in making an embossed overlay sheet which consists of powdered grains of gum mixed with a powdered binder and a powdered astringent both of which having a fusing point substantially lower than that of the gum.
55. 19. An embossing powder for use in the production of an overlay sheet of the character described which is composed of powdered copal gum divided into grains of relatively large size, and powdered dammar gum divided into grains of relatively small size.
60. 20. An overlay sheet for makeready having a rough surfaced resilient embossment, adapted to become indented in the tympan of a printing press, to hold the sheet from displacement and permit temporary depression of the embossment.
65. 21. An overlay sheet for makeready having an embossment of resilient grains of gum forming a roughened surface, adapted to become indented in the tympan of a printing press, to hold the sheet from displacement and permit temporary depression of the embossment.
70. 22. An overlay sheet for makeready having portions thereof embossed with grains of resilient gum embedded in a fused mass of gum which is fused to the sheet.
75. 23. An overlay sheet for use in makeready for printing a picture in which the solid tones of the picture on the sheet are embossed with grains of a resilient gum which are connected by surface fusion to the surface of the sheet.
80. 24. An embossing powder for making overlay sheets for makeready in printing which comprises a plurality of sizes of grains of fusible gum mixed in predetermined proportions, the grains of larger size being adapted to be retained by the more heavily inked portions only of a freshly inked proof sheet, and the size of the smaller grains being

graded to correspond approximately to the weight of the ink on the more lightly inked portions of the sheet, to secure an embossment thereon approximately corresponding to the weight of ink on the different portions thereof.

5 In testimony whereof, I have signed my name to this specification.

ARTHUR L. SMITH.

10

15

20

25

30

35

40

45

50

55

60

65